

Oct. 20, 1936.

J. D. LE VAN

**2,057,661**

**SEAL**

Filed Jan. 27, 1932



Fig. 2.



*INVENTOR*

by JAMES D. LEVAN  
Elmer J. Gorn  
ATTORNEY

## UNITED STATES PATENT OFFICE

2,057,661

## SEAL

James D. Le Van, Belmont, Mass., assignor, by  
mesne assignments, to Raytheon Manufacturing  
Company, Newton, Mass., a corporation of  
Delaware

Application January 27, 1932, Serial No. 589,180

10 Claims. (Cl. 49—81)

This invention relates to seals of the type in which a hermetic seal is established between a metallic electrical conductor and a body of glass.

One of the objects of my invention is to provide a seal between a solid lead-in conductor of relatively large size and a body of glass of such a kind that the temperature of the lead-in conductor may be rapidly raised to a high value without subjecting the glass to fracturing 10 stresses.

The foregoing and other objects of my invention will be best understood from the following description of an exemplification thereof, reference being had to the accompanying drawing, 15 wherein:

Fig. 1 is a cross-sectional view of one end of an electric discharge tube illustrating one embodiment of my invention;

Fig. 2 is an enlarged cross-section taken along 20 Line 2—2 of Fig. 1; and

Fig. 3 is an enlarged perspective view showing an elemental portion of the glass layer on the surface of the lead-in conductor.

In sealing electrical conductors through glass, 25 much work has been done on the problem of obtaining seals of the proper strength under conditions in which the temperature of the lead-in wire remains fairly constant or else changes very slowly. This is a condition which is usually 30 obtained only in electrical devices of comparatively small power rating. When, however, we contemplate using seals on electrical devices of comparatively large power rating, it becomes 35 very difficult to obtain the above temperature conditions for the lead-in-conductor. It is often 40 desirable to change the load on such high power devices very rapidly, sometimes changing from no load to full load in a few seconds. Under 45 these conditions the temperature of the lead-in conductor fluctuates widely and rapidly. Ordinary glass seals having lead-in conductors of a size sufficiently large to carry the loads almost invariably crack under such load and temperature variations. Previous workers in this art 50 have attempted to overcome this disadvantage in various ways. Small lead-in conductors embedded in large thicknesses of glass have been used. Under these conditions, while severe stresses may be set up in the glass close to the surface of the lead-in conductor, yet the large

body of glass in the outer portion of the seal has had sufficient strength to prevent any appreciable stretching of the inner portion of the glass, and therefore has prevented cracking thereof. Obviously in large power devices in which large currents are used, small lead-in conductors are undesirable. In order to utilize large lead-in conductors, use has been made of hollow tubular metal conductors having a thin edge sealed into the glass member. This edge 10 is so thin that under the strains developed, due to heating by electrical currents, the metal in the thin edge reaches its yield point before any great strain is placed upon the glass of the seal. Thus under these strains, the metal in the thin 15 edge actually flows. However, in such seals, the deformation to which the metal is continually subjected ultimately results in the crystallization thereof, whereupon the metal becomes brittle 20 and cracks. I have discovered that a large solid metal lead-in conductor may be sealed in a glass 25 body and the temperature of this conductor may be varied over wide limits within very few seconds without the glass of the seal cracking if the thickness of the layer of glass in contact with the lead-in conductor is made small in comparison with the size of the lead-in conductor. I have further discovered that the thickness of 30 this layer cannot be greater than a definite upper limit, depending upon the materials used and the maximum temperature variations to which the lead-in conductor is subjected.

While the glass layer actually in contact with the metallic lead-in conductor has a tendency 35 to crack, a similar tendency exists in the glass immediately adjacent the point where the contact between the glass layer and the lead-in conductor ceases. This appears to be due to the fact that under rapidly changing temperature 40 conditions, a comparatively large temperature difference exists between the glass in the seal itself and the glass immediately adjacent the point at which contact between the lead-in conductor and the seal ceases. Thus a large temperature gradient exists in the glass at this 45 point, which large temperature gradient sets up excessive strains in the glass. I have eliminated this difficulty by providing means for distributing the temperature difference between the glass in the seal and the rest of the body over a con- 50

siderable length of glass, whereby the temperature gradient at every point in the glass is less than that at which fracturing strains are developed.

Referring to Fig. 1, 1 is the wall of a glass vessel. This glass vessel may be, for example, any type of electron discharge device, such as, for example, an evacuated tube, a gas-filled rectifier, or the like. The vessel is provided with a reentrant stem 2 having a seal 3 at the inner end thereof. Through this seal passes a solid metallic conductor 4 which may be of any suitable metal. This conductor 4 is of a comparatively large diameter, which diameter is preferably in excess of one-tenth of an inch. Of course it will be understood that lead-in conductors of much larger diameter may be used, and also the conductor may be of a somewhat smaller size. The seal 3 comprises a thin layer 5 of glass fused around the conductor 4, whereby a hermetic seal is formed between the conductor and the layer 5. The conductor 4 may be used to conduct electricity to the interior of the glass vessel for any purpose whatsoever. I have illustrated, by way of example, in the drawing the conductor 4 leading to an anode 6. The device would also include a cathode, not shown, and would be connected in some suitable circuit. For example, I have shown a wire 7 connected to the outer end of the lead-in conductor 4. This wire leads to the secondary 8 of transformer 9 having a primary 10 connected to some source of alternating current. A conductor 11 leads from the other end of the secondary 8 to a switch 12, while a third conductor 13 leads to a load device 14. The other terminal of the load device is connected by means of the conductor 15 to the cathode, not shown.

With lead-in conductors of large diameters, I have found that the thickness of the glass layer 5 must be kept below a certain critical value for definite maximum temperature variations of the lead-in conductor 4. I have thoroughly analyzed each of the factors upon which this thickness depends, and have discovered, in accordance with the following analysis, just what this thickness should be in each case. When the diameter of the lead-in conductor 4 is large compared to the thickness of the glass layer 5, an elemental or unit section of the layer 5 in contact with the surface of the conductor 4 approximates a flat plate.

Referring to Fig. 3, I have illustrated such an elemental or unit section, and have shown this section substantially flat. In order to analyze the problem, I designate the metal 4 as a body A and the glass layer 5 on its surface as a body B. The thickness of the layer B may be represented by  $X$ . In order to determine the manner in which the temperature of the glass B varies as the temperature of the metal A varies, we can consider a unit area  $Z$  of the layer B. With the relative sizes as given above, an excellent approximation for purposes of analysis is to consider the thermal capacitance of the block of glass included under the area  $Z$  as being concentrated at the center of said block, this center being at a distance

$$\frac{X}{2}$$

from the surface of the metal body A.

In the table below is given a list of symbols representing constants of the glass layer and the metal body A, which will be used in the following analysis. The values of these constants for

a borosilicate glass and for the metal tungsten which I have utilized in one embodiment of my invention are also given.

The degrees temperature specified are degrees centigrade:

$$I = \text{thermal conductivity for a centimeter cube} = .0027 \frac{\text{cal.}}{\text{sec. deg. cm.}}$$

$$\rho = \text{density} = 2.25 \frac{\text{gm.}}{\text{cm.}^3}$$

$$s = \text{thermal capacity per unit of mass} = .2 \frac{\text{cal.}}{\text{deg. gm.}}$$

$$C = \text{heat capacity} = s \nu \text{ where } \nu = \text{volume of glass element}$$

$$r = \text{thermal resistance for a centimeter cube} = \frac{1}{I}$$

$$R = \text{thermal resistance for 1 cm. cross section to a distance of } \frac{x}{2} = \frac{x}{2I}$$

$$E_A = \text{coefficient of expansion of metal} = 4.5 \times 10^{-6} \text{ for tungsten}$$

$$E_B = \text{coefficient of expansion of glass} = 3.2 \times 10^{-6}$$

$$M_B = \text{Young's modulus for glass} = 623000 \text{ kg./sq. cm.}$$

$$P = \text{tensile strength of glass} = 600 \text{ kg./sq. cm.}$$

Let  $T_A$  = temperature of A

$T_B$  = temperature of B at its center in accordance with our approximation above

Now let us increase  $T_A$  at a certain constant rate  $K$  so that

$$T_A = Kt \quad (1)$$

where  $t$  = time in seconds  
Under these conditions it can be calculated that the maximum temperature difference becomes

$$(T_A - T_B)_{\max} = K(RC) \quad (2)$$

In the above Equation (2)  $RC$  is called the time constant of the glass, and gives the time at which for a sudden application of a definite temperature to the surface of the glass body, the temperature of the glass body will have risen to

$$\left(1 - \frac{1}{e}\right)$$

or 63 per cent. of its final total rise. In this expression  $e = 2.71828$ .

Referring to Fig. 2, the metallic conductor 4 corresponds to body A and the glass seal or layer 5 to layer B, as in Fig. 3.

In order to find the strains and stresses in the glass layer B, due to heating, we can assume that at some temperature  $T_0$ , the glass layer is free from strains.

If we now raise the temperature of A to some value  $T_A$ , strains will be set up in the glass layer which can be expressed as a fractional stretch of the glass layer.

In increasing from  $T_0$  to  $T_A$ , the metal A will undergo a fractional increase in circumference  $I_A$ .

$$I_A = (T_A - T_0) E_A \quad (3)$$

where  $E_A$  = coefficient of expansion of A. Likewise the glass B in increasing from  $T_0$  to  $T_B$  will undergo a fractional increase in circumference  $I_B$ .

$$I_B = (T_B - T_0) E_B \quad (4)$$

where  $E_B$  = coefficient of expansion of B. Then the fractional stretch  $D_B$  of B is the difference between (3) and (4) which is

$$D_B = (T_A - T_0) E_A - (T_B - T_0) E_B \quad (5)$$

In practice  $E_B < E_A$  and therefore

$$E_A = E_B + Y \quad (6)$$

or

$$Y = E_A - E_B$$

5 where  $Y$  is a constant.

Substituting in (5) and simplifying

$$D_B = Y(T_A - T_0) + E_B(T_A - T_B) \quad (7)$$

10 For any value of  $T_A$  we can see that the strain on the glass will be a maximum when  $T_A - T_B$  is a maximum. Taking this maximum value from (2) we get

$$15 E_B(\max) = Y(T_A - T_0) + E_B K(RC) \quad (8)$$

To find the actual stress  $St$  in the glass we multiply the strain by Young's modulus for glass  $M_B$ .

$$20 St(\max) = [Y(T_A - T_0) + E_B K R C] M_B \quad (9)$$

Again referring to the glass section under the area  $Z$ , we can substitute  $R$  and  $C$  in terms of fixed constants of  $B$  and the thickness  $X$  of the glass layer.

$$25 St(\max) = \left[ (E_A - E_B)(T_A - T_0) + E_B K \frac{X^2 S_B}{2I} \right] M_B \quad (10)$$

An examination of the equation yields very valuable information. The factor  $(E_A - E_B)(T_A - T_0)$  is a measure of the final or steady state stress 30 conditions. The factor

$$E_B K \frac{X^2 S_B}{2I}$$

however represents the transient stress condition 35 since its value depends directly on  $K$ , the rate of rise of the temperature  $T_A$  with respect to time (see Equation (1)).

In applying the Equation (10) to a particular case we know the maximum permissible stress 40 that the glass which we are using can stand. We can use any final temperature  $T_A$  such that the steady state stresses are less than the maximum permissible stress and also a certain portion of the maximum permissible stress is left over to provide for the transient stresses. The maximum transient stress while proportional to the first power of the rate of change of the temperature  $T_A$  of the lead-in conductor is also dependent upon the second power of the thickness  $X$  of the 45 glass seal. Thus by keeping this thickness small, we are enabled to use large rates of temperature change. In any case with a definite rate of temperature change, there is a definite upper limit to the thickness which the seal can assume without subjecting the glass to fracturing stresses.

50 As long as our approximation of flat surfaces holds, we can see that the thickness of the glass layer is independent of the size of the lead-in conductor. Thus the same thickness can be used 55 for very large lead-ins as well as smaller ones. This approximation holds good as long as the thickness of the glass layer is small in comparison with the size of the lead-in conductor. However, with lead-ins which are so small that the 60 thickness of the glass layer is not small as compared to the diameter of the lead-in, our approximation of flat surfaces no longer holds and the above analysis no longer gives an accurate picture of the actual conditions. In order to 65 have this approximation hold, the radius of curvature of the surface should preferably be at least of approximately the same value as the thickness of the glass layer. However, it is still more advantageous to use even larger radii of curvature 70 for said surface.

The above analysis can be applied to a seal having any kind of metal and any kind of glass. In a particular instance in which I have used this seal, I utilize a conductor of tungsten about  $\frac{1}{16}$ " in diameter. The wall 1 consisted of a borosilicate glass, such as, for example, that known in the art as "Nonex". The inner part of the stem 2, including the layer 5, was formed of a glass which closely matched the coefficient of expansion of tungsten. For this glass I used 10 another borosilicate glass, which is known in the art as "Corning 705 R". Of course it will be understood that any suitable metal may be used for the conductor 4 and any suitable glass for the seal. We can now apply the analysis to the particular kind of glass and metal as specified above, and calculate the value of  $X$  for this particular example. The tensile strength  $P$  of the glass as taken from the table above is, of course, the maximum permissible stress which can exist in 15 the glass without fracturing it. Thus this value of  $P$  can be substituted in Equation 10 for  $St(\max)$ . We can assume for the sake of simplicity

$$20 T_0 = 0^\circ C.$$

25

which is a condition more adverse than is met with in practice. Therefore a solution on this assumption will give a value of  $X$  which is well within safe limits.

Suppose we wish to operate the lead-in conductor 30 at a temperature of  $600^\circ C.$ , at which temperature it is at red heat, and raise it to this temperature in thirty seconds, we can readily see that these conditions are very extreme, and are such that they have not heretofore been successfully met in practice. From the above conditions our constants for Equation (10) become

$$T_0 = 0^\circ C. \quad T_A = 600^\circ C.$$

$$K = 20$$

$$St_{\max} = 600$$

40

The other constants can be taken from the table of constants given above. Substituting these values in Equation 10 and solving for  $X$ , we get

$$45 X = 19 \text{ cm.}$$

45

This value of  $X$  is the maximum thickness which we can use under the above conditions. In actual practice, of course, we choose a thickness which is not so close to the limiting value. Thus for 50 the particular case given above, we would use a glass thickness of about 1 mm.

It is also interesting to see how the maximum temperature difference between the glass and the tungsten and also the time constant of the glass 55 actually varies for different values of  $X$ .

| X     | Time constant | $(T_A - T_B) \text{ Max.}$ |
|-------|---------------|----------------------------|
| 1 mm. | 833           | $16.66^\circ C.$           |
| 2 mm. | 3.333         | $66.66^\circ C.$           |
| 5 mm. | 20.833        | $416.66^\circ C.$          |

60

It is evident that since increases in the value of  $X$  give such large corresponding changes in time constants, temperature difference and consequently transient strains, we are sharply limited to the safe value of  $X$  as calculated for our 70 glass seal thickness.

While in the specific solution which I have given by way of example above, the constants for tungsten and a borosilicate glass were used, yet for practically any metal and glass seal the con- 75

stants of the materials will be of the order of the constants used above. Therefore the order of thickness of the glass in the seal will be very close to that given by the specific solution above.

5 From the foregoing analysis it will be seen that the radial thickness of the glass wherever in contact with the conductor 4 must be less than a certain predetermined maximum. At the point 16 where the glass leaves contact with the 10 surface of the conductor 4, there is a tendency for the radial thickness of the glass to be greater than the value specified unless special precautions are taken. By making the angle between the 15 surface of the conductor 4 and the surface of the glass at the point where contact ceases small, the radial thickness of the glass at this point can readily be kept within the requisite value. This angle should preferably be of the order of 10 to 20°.

20 While the provision of a thin glass layer 5 wherever in contact with the conductor will prevent the cracking of the seal in this layer itself, the glass still has a tendency to crack somewhere in the region of the point 16 unless additional special precautions are taken. This is due to the fact that the temperature of the glass in the layer 5, due to the thinness of this layer, varies substantially as does the temperature of the lead-in conductor 4. The temperature of the 25 glass not in actual contact with the conductor 4 varies at a much lower rate, due to the fact that its temperature is raised practically entirely by heat conducted through the glass from the layer 5. Thus a sharp temperature gradient would 30 exist at point 16 when the temperature of the lead-in 4 varies at the rapid rate which I use. It can be shown by an analysis similar to that given above that if at any time the temperature gradient in the glass at any point becomes greater 35 than a certain value, fracturing strains would be set up in the glass at that point. In order to decrease this temperature gradient, I provide means to distribute the temperature difference between the glass layer 5 and the rest of the stem 40 45 over a considerable length of glass. In the particular embodiment illustrated, I fill the space between the conductor 4 and the inside walls of the stem 2 with a finely-divided powder 17 of good heat conductivity. This powder may be, 50 for example, a powdered metallic substance, such as, for example, powdered aluminum, copper, tungsten, or the like. In order to retain the powdered material in place, I insert a packing 18 immediately above the powdered material 17. 55 60 This packing is preferably constituted of a metallic foil, such as, aluminum foil, although a cement or sealing compound of some kind could also be used.

65 When current is led through the conductor 4 the temperature of said conductor rises, the temperature of the glass in the seal 3 will rise at approximately the same rate in accordance with the analysis as given above. Since the powdered material 16 is in intimate contact with the glass at the point where it comes out of contact with the surface of the conductor 4 and said powdered material is also in intimate contact with the conductor 4, heat is readily transmitted from each of these elements to said powder. This powder is packed sufficiently densely so that heat is readily transferred therethrough. The heat which passes from the seal 3 and the conductor 4 is transmitted through the powder 16 to the inner 70 75 walls of the enlarged section of the stem 2. Thus

the temperature difference between the walls of the stem 2 and the seal 3 is distributed over a substantial length of glass so that large temperature gradients do not exist at any point in said glass. It will be noted that the walls of the 5 stem 2 are considerably thicker than that of the seal 3. However, the presence of the metal powder 17 in contact with these thicker walls does not introduce any excessive strains on the glass walls of the stem 2, inasmuch as the metallic powder 16 readily yields under any expansions and contractions of the walls of the stem 2, due to temperature increases and decreases.

10 The presence of the metallic powder 17 also eliminates another effect which exists in the 15 vicinity of the point 16. It will be noted that at this point the glass and the metal in the conductor 4 are constrained to expand and contract at substantially the same rate, due to the close bond between the glass and the metal at this 20 point. However, the glass walls of the stem 2 at the point 19 near the outer end of the metallic powder packing have considerable freedom of 25 expansion and movement in all directions so that strains at this point are taken up by said movement without running into the danger of cracking the glass. Thus a considerably greater temperature gradient could exist in the glass at the outer end of the metallic powder packing without fracturing than could exist at the point 16 without cracking the glass.

30 I have constructed a large number of seals of the type described above, using a solid tungsten lead-in rod, the diameter of this rod being about two-tenths of an inch. In many of these seals 35 I have increased the temperature of the conductor by passing current therethrough from room temperature to red heat in a period of about thirty seconds. In each case no fracture of the 40 glass resulted. However, in similar seals without the use of the thin glass layer and the temperature-equalizing arrangement, practically all of the seals cracked.

45 This invention is not limited to the particular details of construction, materials, and processes described, as many equivalents will suggest themselves to those skilled in the art. It is accordingly desired that the appended claims be given a broad interpretation commensurate with the 50 scope of the invention within the art.

What is claimed is:

1. A glass to metal seal comprising a tubular glass member closed at one end, a metal rod sealed directly to the glass through said closed 55 end, leaving a space between said conductor and the side walls of said tubular member, and a material of good heat conductivity placed in said tubular member in intimate contact with said seal and the adjacent side walls of said tubular 60 member and of said conductor.

2. A glass to metal seal comprising a tubular glass member closed at one end, a metal rod sealed directly to the glass through said closed 65 end, leaving a space between said conductor and the side walls of said tubular member, and a non-rigid material of good heat conductivity placed in said tubular member in intimate contact with said seal and the adjacent side walls of said tubular 70 member and of said conductor.

3. A glass to metal seal comprising a rod of metal, a ring of glass completely surrounding said rod and adhering thereto throughout the circumference of said rod, the thickness of said 75

glass ring at every point thereon being not greater than

$$\sqrt{\frac{2 l [P - (E_A - E_B)(T_A - T_0)M_B]}{E_B S_p M_B K}}$$

5 where  $l$ =thermal conductivity for a unit cube of the glass in said layer,

$P$ =tensile strength of said glass,

10  $E_A$ =coefficient of expansion of the metal of said rod,

$E_B$ =coefficient of expansion of said glass,

To=normal temperature of seal at which substantially no strains occur in said glass ring,

TA=maximum steady state temperature which 15 said seal reaches during operation,

$M_B$ =Young's modulus for said glass,

S=thermal capacity per unit of mass of said glass,

$\rho$ =density of said glass,

20 K=rate of temperature change of said metal rod of the order of magnitude of 20° C. per second or more,

the upper edges of said ring being extended to form a glass body surrounding said rod but 25 spaced therefrom, the thickness of said tubular body at the point where its spacing from said rod starts also being of said order of magnitude.

4. A glass to metal seal according to claim 3 in which said metal rod is solid.

30 5. A glass to metal seal according to claim 3 in which the angle between the walls of said

tubular member and the walls of said rod at the point where the spacing between said walls starts is sufficiently acute to prevent an increase in

35 the thickness of the glass at said point as measured in a direction at right angles to the surface of said rod.

6. A glass to metal seal according to claim 3 in which means are provided for distributing the

40 temperature difference between the glass adhering to said metal rod and the rest of the glass in said tubular member, arising as a result of rapid temperature variations in said rod, over an appreciable length of wall of said tubular

45 member, whereby excessive temperature gradients in said tubular member are prevented.

7. A glass to metal seal comprising a rod of metal, a ring of glass completely surrounding said rod and adhering thereto throughout the cir-

50 cumference of said rod, the thickness of said ring at every point thereon being of an order of magnitude of less than about two millimeters, the upper edges of said ring being extended to

55 form a tubular glass body surrounding said rod but spaced therefrom, the thickness of said tubular body at the point where its spacing from said rod starts also being of said order of magni-

tude.

8. A glass to metal seal comprising a solid rod of tungsten having a diameter of the order of five millimeters or more, a ring of borosilicate glass completely surrounding said rod and adhering thereto throughout the circumference of said rod, the thickness of said ring at every point thereon being of an order of magnitude of less than about two millimeters, the upper edges of said ring being extended to form a tubular glass body surrounding said rod but spaced therefrom, the thickness of said tubular body at the point where its spacing from said rod starts also being of said order of magnitude.

9. A glass to metal seal comprising a metal body, a layer of glass adhering to the surface of said metal body, the upper edges of said layer being extended to form a glass body spaced from said metal body, said glass layer at every point thereon being not greater than

$$\sqrt{\frac{2 l [P - (E_A - E_B)(T_A - T_0)M_B]}{E_B S_p M_B K}}$$

where  $l$ =thermal conductivity for a unit cube of the glass in said layer,

$P$ =tensile strength of said glass,

25  $E_A$ =coefficient of expansion of the metal of said rod,

$E_B$ =coefficient of expansion of said glass,

To=normal temperature of seal at which substantially no strains occur in said

30 glass ring,

TA=maximum steady state temperature which said seal reaches during op-

eration,

$M_B$ =Young's modulus for said glass,

S=thermal capacity per unit of mass of said glass,

$\rho$ =density of said glass,

K=rate of temperature change of said

40 metal rod of the order of magni-

tude of 20° C. per second or more,

the angle between the walls of said glass body and the walls of said metal body at the point where the spacing between said walls starts being sufficiently acute to prevent an increase in the thickness of the glass at said point as measured in a direction at right angles to the surface of said metal body.

10. A glass to metal seal comprising a tubular glass member closed at one end, a metallic rod sealed directly to the glass through said closed end, a powdered metal packed in the inside of said tubular member in contact with said seal, said conductor and the inner side walls of said tubular member, and means for retaining said powdered metal in intimate contact with all of said elements within said tubular member.

JAMES D. LE VAN.